

## UNITED STATES PATENT OFFICE

2,233,426

## LUBRICANT

John G. McNab, Roselle, N. J., assignor to Standard Oil Development Company, a corporation of Delaware

No Drawing. Application October 14, 1938,  
Serial No. 234,899

12 Claims. (Cl. 252—36)

The present invention relates to improved lubricants and especially to oils for the lubrication of automotive engines, and particularly Diesel engines. The invention will be fully understood from the following description.

During the past several years it has been found desirable to add certain polyvalent metal soaps to lubricants, especially such lubricants as are used for automotive engines of the Diesel type. The function of these soaps is complex but the effect is mainly one of maintaining a clean engine condition. The various soaps have peculiarities in behavior depending on the particular metals and to some degree the acid radicals with which they are combined. Certain of the soaps are completely insoluble and others, while soluble, cause gelling of the oil. Still others are capable of giving clean engines, but do not appear to be able to reduce engine wear or perhaps even cause excessive engine wear. Thus the various soaps, while their functions may in some cases overlap, are not equivalents in some certain respects.

It has now been found that certain mixed soap compositions are very much superior to compositions containing a single soap. Of the various soaps to be under consideration here, there appear to be three general groups; the first comprises calcium and magnesium soaps which appear to be interchangeable, although they may be used together if desired. The second type of soap is that of aluminum and the third of nickel. The results produced by these various soaps as stated above overlap to some extent, but nevertheless they do not appear to be full equivalents. Improved results are obtained by using a mixture of soaps from any two of these groups, or by using the three types of soap in combination. Thus either a nickel or an aluminum soap may be used along with either calcium or magnesium and the nickel-aluminum combination is also good. Furthermore, improved results have been obtained by use of three soaps, nickel, aluminum and calcium or magnesium.

It has been stated that the type of acids used is important. Any of the fatty acids may be employed but it is preferable to use predominantly saturated fatty acids with melting points below 50° C. The higher melting acids such as stearic and palmitic are less desirable because their soaps have a tendency to be less soluble than those of acids having melting points below 50° C., such as capric, lauric and the like. Various mixed acids may be used such as are obtained from the commercial fats or may be made up synthetically, and it is found that if a substantial portion of unsaturated acids be present, say from about 10 to 30%, oil solubility is more readily obtained. Unsaturated acids such as oleic or erucic can also be used alone. Another type of acids that may be employed is that produced by

low temperature oxidation of paraffin wax with air, preferably using catalysts. Highly refined oils may be oxidized in the same way, for example, highly solvent extracted oils or hydrogenated oils, but the most suitable product appears to be the so-called oxidized acids which are obtained from sweater oil. This oil is sweated from petroleum waxes and is oxidized catalytically with air at temperatures from about 110 to 160° C.

Naphthenic acids such as those obtained from Venezuelan, Colombian, Gulf Coast, and Roumanian crudes may also be used in making the soaps.

In manufacturing the soaps, the best procedure is to first obtain a soda or potash soap of the particular organic acid or mixture of acids and then prepare the polyvalent metal soap mixture from the soda or potash soap by double decomposition using water soluble salts of the polyvalent metals, for example chlorides or nitrates. In some instances, the polyvalent soaps may be prepared separately and then mixed together, but it is generally preferable to make a mixture of the polyvalent soaps directly by co-precipitation and this is particularly useful when calcium soaps are employed because they have a tendency to be less soluble than the other metal soaps and the co-precipitation method produces materials which are freely soluble.

The amount of the soap may vary somewhat depending on the particular soaps employed and the service in which they are to be used, but the total amount of the polyvalent metal soap varies in general from about  $\frac{1}{10}$  to  $3\frac{1}{2}\%$  of the oil. The various soaps may be used in equal proportions, but good results are obtained over a fairly large range of variation in proportions. It is preferable to provide that each of the two or more soaps is present in not less than  $\frac{1}{10}$  of the total soap. Thus if 3% of the total soap is employed, the mixture may contain from about .3 to 2.7% of the aluminum soap with from 2.7 to .3% of calcium, magnesium or nickel soap.

It is found desirable to use soap mixtures which are substantially free from non-saponaceous ingredients such as free acids, esters, lactones, lactides, and the like and this may be accomplished in various ways, but the best method is by extracting the soap mixtures with oxygen-containing solvents such as alcohols, ketones, and the like in which the polyvalent soaps are relatively insoluble.

In spite of what has been said in the paragraph above, it has been found desirable to add small amounts of certain specific acids to the soap mixtures, but these acids are not of the preferred type used in manufacturing polyvalent soap. The best acid to be added appears to be a good grade of stearic acid, but similar high molecular weight

saturated acids may be employed instead. This acid is added to the oil or to the soap mixture after extraction and the amount may vary from about .1 to 1% of the total mixture.

- 5 The soaps may be added to any type of mineral oil, that is to say lubricating oils of naphthenic, paraffinic or mixed base crudes, but particularly to the distillates of naphthenic crudes and these compositions are especially desirable 10 for the lubrication of Diesel engines. The oils are preferably well refined having viscosities from 45 to 65 seconds Saybolt at 210° F., and it is preferred that they have pour points of 0° F. or below; whether obtained naturally or by de- 15 waxing or by the use of pour depressants is not important. The essential ingredients of the present composition are the two or more polyvalent soaps of the types mentioned above and the hydrocarbon oil, but other ingredients may 20 be employed such as sludge dispersing agents, oxidation inhibitors, thickening agents, sulfur or phosphorus containing compounds, and the like.

*Examples*

- 25 Lubricating oils made from naphthenic lubricating distillate having a viscosity of about 55 seconds at 210° F. Sample 1 contained 1% of an aluminum soap of an oxidized sweater oil acid and .5% of free stearic acid. Sample 2 30 contained 1% of a calcium soap of the same oxidized sweater acids and .5% of naphthenic acid which was used to solubilize the calcium sweater oil acids soap. Sample 3 contained .75% of a mixture of aluminum and calcium sweater 35 oil acids soaps in equal proportions. This mixture was prepared by co-precipitation of the said soaps by addition of aluminum and calcium chlorides to the soda soap of the oxidized sweater oil acids. The blend also contained .5% added 40 free stearic acid.

Each of the three samples described above was subjected to a test over long periods in a Caterpillar single cylinder Diesel engine under comparable running conditions. After each 45 test the pistons were taken down and examined carefully and a demerit rating was assigned to each part depending on its condition, for example, to the rings, slits, and grooves, filter, piston skirt, and liners. In considering these demerit numbers, it should be borne in mind that the lower numbers indicate superior condition. The demerit numbers were then weighted to obtain an overall demerit for the piston as a 50 whole. The amount of oil used was measured as well as the wear on the liner. All of these 55 data are assembled in the following table:

The overall demerit rating is much better and only in one comparison is it inferior to either of the other samples. This is in respect to the sharpness of the ring edge, but it is clear that this is not of very great importance and is much 5 overshadowed by the improved condition of the slits, grooves, etc., the decrease in the varnish and the improved filter condition.

This invention is not to be limited by any specific examples which have been presented 10 herein solely for the purpose of illustration, but only by the following claims, in which it is desired to claim all novelty inherent in the invention.

I claim:

1. An improved crankcase lubricating composition comprising a mineral lubricating oil and small amounts of polyvalent metal soaps selected from at least two of the groups of aluminum, nickel, and the alkaline earth soaps the total 20 amount of soaps present being from  $\frac{1}{10}$  to 3½% of the oil, and the amount of soap from any one of the three groups being at least 10% of the total amount of soap present.

2. Lubricant according to claim 1, in which 25 the total soap amounts to from  $\frac{1}{10}$  to 3½% and is prepared by co-precipitation of the two soaps by reaction of alkali metal soaps with water soluble salts of the said polyvalent metals.

3. An improved lubricant for Diesel engines 30 comprising a mineral lubricating oil and  $\frac{1}{10}$  to 3½% of mixed soaps, the said soaps being prepared from soda soaps of organic acids by co-precipitation with water soluble salts of aluminum and a metal selected from the group consisting of calcium and magnesium the amount of each soap in the lubricant being at least 10% 35 of the total amount of soaps present.

4. Lubricating oil according to claim 3 in which the soap is prepared from oxidized sweater oil 40 acid.

5. An improved lubricant for Diesel engines comprising a mineral lubricating oil and  $\frac{1}{10}$  to 3½% of mixed soaps, the said soaps being prepared from soda soaps of organic acids by co-precipitation with water soluble salts of nickel 45 and a metal selected from the group consisting of calcium and magnesium the amount of each soap in the lubricant being at least 10% of the total amount of soap present.

6. Lubricating oil according to claim 5 in which the soap is prepared from oxidized sweater oil acid.

7. Lubricant according to claim 1, in which the total soap content is from  $\frac{1}{10}$  to 3% and is prepared by co-precipitation of the two soaps by re- 55

*Caterpillar single cylinder engine tests*

| Sample No. | Eng. No. | Run No. | Hours | Demerits               |                 |                       |     |      |             |                 |                  |            |      | Oil cons. B. H. P. hrs./gallon | Liner wear per 1000 hrs. |      |
|------------|----------|---------|-------|------------------------|-----------------|-----------------------|-----|------|-------------|-----------------|------------------|------------|------|--------------------------------|--------------------------|------|
|            |          |         |       | Overall piston demerit | Ring edge sharp | Ring zone cleanliness |     |      | Car-<br>bon | Skirt and liner | Varnish on skirt | Oil filter |      |                                | Max.                     | Avg. |
| Slits      | Grooves  | SGLS*   |       |                        |                 |                       |     |      |             |                 |                  |            |      |                                |                          |      |
| 65         |          |         |       |                        |                 |                       |     |      |             |                 |                  |            |      |                                |                          |      |
| 1.....     | C-2      | 3       | { 500 | 1.35                   | 0.17            | 0.0                   | 3.1 | 1.72 | 4.6         | 0.92            | 1.0              | 2          | 3200 | 0.0046                         | 0.0015                   |      |
|            |          |         | 1000  | 2.00                   | 0.67            | 0.5                   | 4.5 | 2.52 | 5.0         | 1.92            | 0.8              | .5         | 3500 | 0.0045                         | 0.0016                   |      |
| 2.....     | C-1      | 17      | 500   | 2.25                   | 0.17            | 3.0                   | 4.2 | 3.03 | 4.8         | 3.33            | 4                | 4          | 3400 | 0.0028                         | 0.0012                   |      |
| 3.....     | C-2      | 8       | { 500 | 1.13                   | 0.25            | 0.0                   | 2.3 | 1.28 | 4.4         | 0.67            | 0.25             | 1.0        | 270  | 0.0036                         | 0.0016                   |      |
|            |          |         | 1000  | 1.48                   | 1.00            | 0.25                  | 3.6 | 2.01 | 4.3         | 0.67            | 0.00             | 2.0        | 3545 | 0.0022                         | 0.0009                   |      |

\*Cleanliness of ring slits, grooves, lands, and sides.

From the above data it is clear that the oil containing both the calcium and the aluminum soap, Sample 3, is much superior to either of the blends in which the single soaps are used.

action of alkali metal soaps of naphthenic acids with water soluble salts of the polyvalent metals.

8. An improved lubricant for Diesel engines comprising a mineral lubricating oil and  $\frac{1}{10}$  to 75

3½% of mixed soaps, the said soaps being prepared from soda soaps by co-precipitation with water soluble salts of nickel, aluminum, and a metal selected from the group consisting of calcium and magnesium the amount of each soap in the lubricant being at least 10% of the total amount of soap present.

9. Lubricant according to claim 1, in which the mineral lubricating oil present, is a refined mineral oil having a viscosity of 45 to 65 seconds Saybolt at 210° F. and a pour point at least as low as 0° F.

10. Lubricant according to claim 1 in which the soap-forming acidic material has been substantially freed from non-saponaceous ingredients such as free acids, esters, lactones, lactides and the like.

11. An improved crankcase lubricant for Diesel engines comprising a major proportion of naphthenic lubricating oil distillates having a viscos-

ity of about 45 to 65 seconds Saybolt at 210° F., into which has been incorporated from ¼ to 3½% of mixed soaps of polyvalent metals selected from at least two of the groups aluminum, nickel and alkaline earth soaps, said soaps being prepared from saturated fatty acids having a melting point below about 50° C. the amount of each soap in the lubricant being at least 10% of the total amount of soap present.

12. An improved lubricant for Diesel engines comprising essentially a naphthenic lubricating oil distillate having a viscosity of about 45 to 65 seconds Saybolt at 210° F. and a pour point at least as low as 0° F., into which has been incorporated about 0.75% of a mixture in equal proportions of aluminum and calcium soaps of acids prepared by the oxidation of sweater oil, said lubricant also containing about 0.5% of added free stearic acid.

JOHN G. McNAB. 20